

# UNITED STATES PATENT OFFICE.

FRED. A. PAGE, OF PHILADELPHIA, NEW YORK.

## STOVE-POLISH.

SPECIFICATION forming part of Letters Patent No. 250,098, dated November 29, 1881.

Application filed August 15, 1881. (No specimens.)

*To all whom it may concern:*

Be it known that I, FRED. A. PAGE, of the town of Philadelphia, county of Jefferson, and State of New York, have invented a new and useful Compound Liquid Polish to be used for polishing stoves and other iron articles of manufacture, of which the following is a specification.

Said compound is described as follows, and is composed of the following-named articles or ingredients, mixed together in about the following quantities and proportions, viz: one gallon benzine, one pound black-lead, one-fourth pound rosin, two ounces lamp-black, 15 one ounce borax, one ounce alum. The black-lead, rosin, lamp-black, borax, and alum are ground and mixed together with the benzine.

The compound may be applied with a brush, sponge, or other soft substance, and the coating is then rubbed with a dry brush until pol-

ished. It makes a very desirable polish, durable, and of great luster.

The elements or ingredients of my compound liquid polish have been used before in such compounds separately, and some of them together; but I am not aware that they all have been used together to form a compound of this kind. 25

I claim as my invention and desire to secure by Letters Patent of the United States— 30

The composition of matter herein described to be used for polishing stoves and other iron articles of manufacture, consisting of benzine, black-lead, rosin, lamp-black, borax, and alum, substantially in the proportions specified.

FRED. A. PAGE.

Witnesses:

A. C. COMSTOCK,  
J. C. MASHER.